

Sept. 16, 1958

C. G. GOETZEL ET AL

2,852,367

METHOD OF MANUFACTURING HEAT RESISTANT SINTERED ARTICLES

Filed Aug. 27, 1954



FIG. 1



FIG. 2.

INVENTORS

Claus G. Goetzel, Nicholas J. Grant  
Jack A. Yoblin & Leonard P. Skolnick

*Paul M. Nichols*

ATTORNEY

1

2,852,367

**METHOD OF MANUFACTURING HEAT RESISTANT SINTERED ARTICLES**

Claus G. Goetzl, Yonkers, N. Y., Nicholas J. Grant, Winchester, Mass., and Jack A. Yoblin, Bronx, and Leonard P. Skolnick, New York, N. Y., assignors to Sintercast Corporation of America, Yonkers, N. Y., a corporation of New York

Application August 27, 1954, Serial No. 452,595

5 Claims. (Cl. 75—201)

The present invention relates to heat resistant metal products and more particularly to a reinforced heat resistant metal product capable of sustaining high strength properties and high resistance to creep at elevated temperatures above 800° C. and up to 950° C. and higher for prolonged periods of time.

It is well known that considerable progress has been made in recent years in the development of wrought nickel- and cobalt-base "super-alloys" for use in the production of power plant components for high powered thermal engines such as turbines, rockets, jets and the like. While these alloys have added measurably to the scientific development of such engines, increased operating temperatures of the more recently developed thermal engines to improve their power rating have placed considerable burden on these alloys. It was found that these alloys had definite temperature limitations in that they tended to soften and creep appreciably at temperatures above 900° C.

The typical wrought super-alloy generally comprises a wrought solid solution alloy containing chromium and at least one metal of the iron group as essential alloying ingredients together with hardening elements to stiffen the alloy for use at high temperatures. Generally, the stiffening may be achieved in several ways: (1) by hardening the solid solution matrix by employing such matrix hardening elements as molybdenum, tungsten, columbium, etc., (2) by employing special elements capable of forming compounds of low solubility which precipitation-harden the alloy, for example titanium, aluminum, zirconium, etc., (3) by employing other elements which form a second phase upon solidification which hardens the alloy, etc. The hardening by the second method is achieved by heat treatment and may be employed to augment the hardening of the first method. Generally, most of the wrought super-alloys are susceptible to precipitation hardening. The precipitation hardening elements in the alloy are taken into solid solution by heating the alloy to a high solution temperature, for example 1000° C. to 1250° C., followed by rapid cooling to keep the precipitation hardening elements in solution. The precipitation hardening is then achieved by reheating the alloy at a lower temperature, for example within the range of about 550° C. to 850° C., for a time sufficient to produce a critical dispersion of a fine precipitate throughout the matrix which is generally invisible, even at a magnification of 2000 times and higher when achieving maximum benefit. Such alloys in the hardened condition exhibit improved resistance to creep at elevated service temperatures up to about 900° C. However, at higher temperatures, the alloys tend to soften due to two effects. If the service temperature is in the neighborhood of about 850° to 900° C. and slightly higher, the alloys tend to soften due to over-aging. This phenomenon is believed to be due to a coalescence of the fine precipitate to large, coarse particles which is generally accompanied by a falling off in hardness and hence lower resistance to creep. Moreover, when the service temperature is in the

2

neighborhood of 1000° C. to 1100° C. and higher, the precipitate begins to go into solid solution and the alloy softens much as a regular high temperature solution temperature softens or anneals a precipitation hardened super-alloy. When the alloy softens because of the foregoing reasons, it loses its ability to sustain high static and/or dynamic stresses and generally deforms. Furthermore, such alloys tend to form abnormally large grains at the high temperatures and generally become embrittled. Because 10 tolerances and clearances of rotating and stationary members of thermal engines must be kept extremely small, any variation from normal creep can be dangerous and lead to serious damage of the power plant, even to the extent where the whole engine may be temporarily stalled or possibly totally destroyed.

In an attempt to overcome the foregoing difficulties, super-alloys were proposed with higher amounts of hardening elements, e. g. carbon, to further stiffen them so as to increase their sustaining power at elevated temperatures. While this was helpful to a certain extent, the stiffened alloys generally had lower ductility which was accompanied by a low resistance to impact. Moreover, the alloys could not be worked easily and generally were subject to cracking during the hot working operations. 25 This was especially true when the super-alloys contained particularly high amounts of matrix hardening elements, e. g. tungsten, molybdenum, etc., and high amounts of precipitation-hardening elements such as titanium, aluminum, zirconium, etc. Although many attempts were 30 made to overcome the foregoing difficulties, none, as far as we are aware, was entirely successful when carried into practice commercially.

We have now discovered that heat resistant super-alloys with improved sustaining power at elevated temperature, especially sustained resistance to creep at elevated temperatures, well above 800° C. and even above 950° C., or 1000° C., in combination with high resistance to impact, can be produced by employing substantial amounts of a hardening constituent which would normally 35 embrittle the alloy. By employing the hardening constituent in a special manner, the alloys of the invention are capable of maintaining their stiffness at elevated temperatures which normally cause similar alloys outside the invention to soften and creep substantially.

40 It is the object of the present invention to overcome the limitations inherent in the presently available heat resistant nickel- and cobalt-base alloys and thereby produce an entirely new type of material which combines high ductility with improved resistance to thermal and mechanical shock and to creep at elevated temperatures.

The advantages of the invention will become apparent from the following description taken in conjunction with the accompanying drawing which shows microstructures of heat resistant metal products within the scope of the 45 invention as illustrated by Figs. 1 and 2.

Generally speaking, the present invention contemplates the use of a slip inhibiting compound having a high melting point and being characterized by a low degree of solubility in the solid solution matrix of the 50 heat resistant alloy in which it is contained. The compound also behaves as a recovery inhibitor, that is, it acts as a deterrent to recrystallization and to abnormal grain growth. The compound is stable and does not decompose substantially at elevated temperatures and, when uniformly dispersed throughout the matrix of a heat resistant alloy, the alloy is capable of sustaining its mechanical properties for prolonged periods of time at elevated temperatures that normally cause similar heat resistant alloys to soften and creep appreciably. It is essential that the 55 alloy with the slip and recovery inhibitor be produced by powder metallurgy as ordinary melting techniques will not produce the results of the invention. Compounds suitable 60

70

as inhibitors are characterized by being slightly soluble in the solid solution matrix of the heat resistant alloy at elevated fabrication temperatures but yet insoluble enough to enable their use as slip and recovery inhibitors at high temperatures. It is essential that the high melting point slip and recovery inhibitors be slightly soluble so that they will bond securely with the matrix alloy, otherwise if the inhibitors have no solubility in the matrix alloy, poor bonding results which gives rise to internal cracks and structural defects under stress during fabrication or use. Excessive solubility, on the other hand, tends to decrease the stability of the entire structure at elevated temperatures, leading to a gradual reduction in service life due to coalescence of and consequent reduction in the effectiveness of the slip and recovery inhibiting phase. The slip inhibitors contemplated comprise mainly the carbides, borides, silicides and nitrides of titanium, zirconium, columbium, tantalum, hafnium and vanadium, and also the disilicides of molybdenum and tungsten.

In carrying the invention into practice, the hard phase is employed in amounts ranging from about 5% to 20% by volume, substantially the balance by volume being the heat resistant matrix alloy.

The heat resistant matrix alloy contemplated by the invention comprises about 5 to 30% by weight of chromium and up to about 25% by weight of iron, substantially the balance of the alloy being at least one metal selected from the group consisting of up to about 90% nickel and up to about 70% cobalt, the sum of the nickel and cobalt contents being at least about 40% of the total alloy composition and preferably at least 50%.

The expressions "substantially the balance" or "balance" or "remainder" as employed herein do not exclude the presence of other elements in amounts which do not adversely affect the basic characteristics of the alloy. Thus, the heat resistant matrix alloy may contain, in addition to chromium, either tungsten or molybdenum, or both, in amounts not inconsistent with forming a substantially ductile matrix. This is also true for other elements which may be present such as columbium, tantalum, titanium, aluminum, etc., provided these and the other elements are not present in amounts that produce phases detrimental to the properties of the alloy, such as the brittle sigma phase in chromium-bearing alloys or other phases. As those skilled in the art will readily understand, small amounts of other elements may be present either incidentally or as regular additions such as manganese, silicon, boron, etc. With respect to the carbon and nitrogen contents, these elements generally do not exceed about 0.25% and about 0.1%, respectively, and preferably should be maintained as low as possible.

In producing reinforced heat resistant metal products in accordance with the invention, the finely divided slip and recovery inhibitor compound is mixed with the finely divided heat resistant matrix metal and shaped to a desired configuration which may be accomplished by pressing the powder mixture in a die mold by employing a pressure varying from about 30 to 150 tons per square inch. The resulting body is then sintered at an elevated temperature to consolidate it sufficiently so it can be subsequently hot worked. Generally, the sintering is conducted at a temperature of at least about 1100° C. but not exceeding about 5° below the point of incipient fusion at a subatmospheric pressure generally not exceeding about 100 microns and preferably not exceeding about 50 microns. It is preferred that the sintering be carried out in two stages, the first stage being carried out at a temperature ranging from about 1100° C. to 1125° C. with the second stage at about 5° C. to 100° C. below the temperature of incipient fusion and preferably 25° C. to 100° C. below. When employing the second stage of sintering, it is preferred that a subatmospheric pressure not exceeding about 0.1 micron be employed. The sintered body is then hot worked, for example by hot extrusion, forging, swaging, etc., until its cross-section has been reduced at least 50% and preferably at least 90% to 95% so that sub-

stantially all of the voids have been eliminated after which the hot worked body is fabricated into the finished product.

As has been pointed out hereinbefore, it is essential that powder metallurgy be employed in producing the reinforced metal product of the invention. In order to obtain a satisfactory dispersion of the hard phase in the relatively soft matrix, it is necessary that the base or matrix metal be employed as a fine powder, the maximum particle size not exceeding 40 microns and preferably not exceeding 5 microns, whereas the slip and recovery inhibitor phase should be of even finer particle size, e. g. not exceeding 10 microns, and preferably not exceeding two or even one micron in particle size. When a commercial nickel-chromium alloy comprised of about 80% nickel and 20% chromium is employed as the matrix, the fine powder can be obtained by mechanical comminution or milling the alloy, or preferably by the reduction of nickel and chromium oxide powder mixtures in the proper proportion. Since it is important that the powder be as free from oxygen as possible, reduction of the oxide mixture by the hydride process is preferred. As for the hard slip and recovery inhibitor phase, e. g. titanium carbide, the ultra-fine powder can be obtained by prolonged ball milling in carbide-lined ball mills, using cemented tungsten carbide balls. Milling times are preferably in the order of 120 hours and in a medium such as xylene, trichlorethylene or carbon tetrachloride.

The two powdered ingredients are blended in a volumetric proportion of from 80-95% of the relatively soft matrix metal powder and 5-20% by volume of the ultra-fine hard slip inhibitor powder. When the 80-20 nickel-chromium base or matrix alloy is employed with titanium carbide as the slip inhibitor phase, the weight proportions would be about 85% to 97% of the alloy and about 15% to 3% of titanium carbide.

The mixture is ball milled in a carbide-lined mill for about 120 to 168 hours in a commercial solvent such as carbon tetrachloride. After drying, the mixture is then briquetted or shaped at room temperature into ingots at pressures ranging from about 30 to 150 t. s. i. (tons per square inch). The ingots are then sintered in two stages, first at about 1100 to 1125° C. under a moderate vacuum of the order of 50 microns Hg column. In the case of a matrix of nickel-chromium alloy and a slip inhibitor of titanium carbide, strong out-gassing takes place at this temperature due to a strong reaction between the nickel-chromium alloy and the titanium carbide. A small ingot 3" in length and 1/2" square requires up to 6 hours for complete degassing by means of a mechanical vacuum pump, the exact time depending on the proportion and fineness of the nickel-chromium alloy and the titanium carbide powders. With the completion of this first sintering stage, the ingot is ready for the second stage which may either directly follow the first stage or which may follow an intermediate cooling under vacuum to room temperature. The second stage has the purpose of shrinking and consolidating the ingot to a density approaching as nearly as possible that of the solid body. The treatment is carried out at a temperature ranging from about 5° C. to 100° C. below the temperature of incipient fusion and preferably from 25° C. to 100° C. below. The latter is about 1285° C. for a composition comprising about 96% by weight of the 80-20 nickel-chromium alloy and 4% by weight titanium carbide. It is about 1250° C. for a composition comprising about 90% by weight of the nickel-chromium alloy and 10% by weight of titanium carbide. The subatmospheric pressure during this second phase of the treatment must be appreciably lower than the first. It is preferred that it not exceed about 0.1 micron Hg column. The period of this second stage sintering is dependent on the size of the ingot: 4 hours being sufficient for a small ingot of 3 inches in length and 1/2 inch square cross-section to produce a material having not more than 6% void space left.

The thus-sintered ingot has excellent physical proper-

ties, namely, a modulus of rupture in the order of 300,000 p. s. i., a yield point of 200,000 p. s. i., an impact resistance at room temperature and at 1000° C. of over 50 inch-pounds for a  $\frac{3}{16}$ " cross-section as measured by the Micro Charpy Impact test. In order to produce useful articles from the novel material, such as turbine blades, nozzles, and the like, the ingot is then hot worked, for example by hot swaging, forging or extrusion, until it has been reduced in cross-section by at least 50% and preferably 90% to 95%, until substantially all residual voids have been eliminated and an optimum dispersion of the inhibitor phase is obtained. The material is then ready for conventional metal working and fabricating processes such as forging, rolling, cutting, trimming, welding and brazing.

Further details concerning the invention become apparent from the following examples.

*Example I*

About 96% by weight of substantially minus 325 mesh 20 80-20 nickel-chromium alloy powder is mixed with about 4% by weight of substantially minus 2 micron high purity titanium carbide.

The size analysis of the nickel-chromium alloy powder used as established by a microscopic count was as follows:

Less than 2 microns—about 16%

About 2 microns to 5 microns—about 44%

About 5 microns to 10 microns—about 28%

About 10 microns to 44 microns—about 12%

Greater than 44 microns—about 0%

The size analysis of the titanium carbide used which is generally much finer is as follows:

Less than 1 micron—about 95%

About 1 micron to about 2 microns—about 5%

Maximum particle size about 2 microns

Average particle size about 0.5 micron

The mixture was ball milled in a carbide-lined mill using carbide balls in a liquid media comprising carbon tetrachloride. The procedure used was to fill the mill one-third full with balls, and to fill the interstices between the balls with the titanium carbide reinforced nickel-chromium metal powder mixture. Carbon tetrachloride was added to the half-way mark in the mill. The mixture was ball milled for about one week (168 hours).

The powder was dried and then compacted into test specimens. The test specimens were 3 inches long and  $\frac{3}{16}$  inch wide. Fifty grams of powder were used, and the compacting pressure was 50 t. s. i. The test specimens obtained were about 72% dense.

The titanium carbide reinforced metal powder specimens were sintered on a beryllium oxide support in an ultra high vacuum furnace. The specimen and support were degassed at pressures from 100 down to 50 microns at temperatures up to about 1000° C. The furnace was maintained at 1125° C. until the pressure dropped below 20 microns. This degassing took approximately six hours. At this point, the high vacuum diffusion pumps were turned on and a vacuum of better than 0.1 micron was maintained throughout the remainder of the sintering operation. The temperature was raised (always keeping the vacuum better than 0.1 micron) until 1270° C. was reached. This was 15° C. less than the incipient fusion point of the alloy. Once the furnace had reached 1270° C. and the vacuum was better than 0.1 micron, the specimen was sintered at these conditions for four hours. The furnace was vacuum cooled.

The final density of the specimen was 8.15 g./cc. (grams per cubic centimeter), which corresponds to 97.5% of the theoretical density of the composite (based on the assumption that there is substantially no solubility between the components). The sintered material was then hot worked in accordance with the invention to assist in obtaining full densification and an optimum dispersion of the slip and recovery inhibitor phase.

*Example II*

The method of Example I was employed except that about 7% titanium carbide by weight all finer than 2 microns was added to about 93% by weight of the 80-20 nickel-chromium alloy powder all finer than 40 microns and the final sintering temperature was conducted at about 1255° C. (fusion point of this alloy 1270° C.). The final density was 7.67 g./cc. which corresponds to 94% of the theoretical density, assuming no solubility between the components. The sintered reinforced product was then hot worked in accordance with the invention, for example swaged, in order to obtain substantially full densification and an optimum dispersion of the slip inhibitor phase.

*Example III*

The method of Example I was employed except that about 10% by weight of titanium carbide (minus 2 microns) was added to 90% by weight of the 80-20 nickel-chromium alloy of less than 40 microns in size. The final sintering temperature was conducted at about 1235° C. (fusion point of this alloy 1250° C.). The final density was 7.4 g./cc. which corresponds to 94% of the theoretical density (assuming substantially no solubility between the components). The sintered reinforced product was thereafter hot worked for the reasons given in Examples I and II.

*Example IV*

30 The method of Example I was employed except that about 7% titanium carbide by weight, all finer than  $\frac{1}{2}$  micron, was added to about 93% by weight of 80-20 nickel chromium alloy powder, all finer than 5 microns, and the final sintering temperature was conducted at about 1255° C. (the fusion point for this alloy is 1270° C.). The final density was 7.70 grams per cubic centimeter which corresponds to 94.5% of the theoretical density, assuming no solubility between the components. The sintered reinforced product was thereafter hot-worked in accordance with the invention for the reasons given in Examples I and II.

*Example V*

45 About 90% by weight of substantially minus 325 mesh 60-32-6 cobalt-chromium-tungsten alloy powder was mixed with about 10% by weight of substantially minus 10 microns zirconium carbide. The mixture was dry-blended in a rotating mill for about 24 hours. The powder was compacted into test specimens. The test specimens were 2" long  $\times \frac{3}{16}$ " wide. About 10 grams 50 of powder were used and the compacting pressure was about 50 t. s. i. The test specimens obtained were about 70% dense. The zirconium carbide reinforced metal powder specimens were sintered on a beryllium oxide support in an ultra-high vacuum furnace. The specimens and supports were degassed at pressures less than 50 microns at temperatures up to approximately 1000° C. The furnace was maintained at about 1000° C. until the pressure dropped below 20 microns. This degassing took approximately 4 hours. At this point the high vacuum diffusion pumps were turned on and a vacuum of better than 0.1 micron was maintained throughout the remainder of the sintering cycle. The temperature was raised (always keeping the vacuum better than 0.1 micron) until 1350° C. was reached. This is about 20° C. 60 less than the incipient fusion point of the alloy. Once the furnace had reached 1350° C. and the vacuum was less than 0.1 micron, the specimen was sintered at these conditions for approximately 4 hours and the furnace was vacuum cooled.

70 The final density of the specimen was 7.4 grams per cubic centimeter which corresponds to 90.0% of the theoretical density of the composite disregarding limited solid solubility between the components. However, metallographic examination revealed less than 2% porosity. 75 The product was then hot-worked in accordance with the

invention to assist in obtaining full densification and an optimum dispersion of the slip and recovery inhibitor phase.

*Example VI*

The method of Example V was employed except that about 10% by weight of zirconium boride (all finer than 5 microns) was added to about 90% by weight of 80-14-6 nickel-chromium-iron-alloy powder (all minus 400 mesh). The final sintering temperature was about 1100° C. which is approximately 20° C. less than the fusion point of this alloy. The final density was 7.4 grams per cubic centimeter which corresponds to 90.4% of the theoretical density disregarding limited solid solubility between the components. However, metallographic examination revealed less than 2% porosity. The sintered, reinforced product was then hot-worked in accordance with the invention for the reasons given in Example V.

*Example VII*

The method of Example VI was employed except that about 10% by weight of titanium boride (all minus 5 microns) was used as the slip and recovery inhibitor phase. The sintering temperature for this composite was 1150° C. which is about 15° less than the fusion point of this alloy. The final density was 7.02 grams per cubic centimeter which corresponds to 90.5% of the theoretical density disregarding limited solid solubility between the components. However, metallographic examination revealed less than 2% porosity. The sintered reinforced product was then hot-worked in accordance with the invention for the reasons given in Example V.

*Example VIII*

The method of Example V was employed except that 10% by weight of titanium nitride (all finer than 5 microns) was blended with about 90% by weight of an alloy which consisted of 20% cobalt, 20% chromium, 2.3% titanium, 0.8 aluminum, and the balance nickel. This alloy was substantially all minus 400 mesh. The final sintering temperature was conducted at approximately 1380° C. which is about 20° C. less than the fusion point for this alloy. The final density was 7.70 grams per cubic centimeter which corresponds to 91.0% of the theoretical density disregarding limited solid solubility between the components. However, metallographic examination revealed less than 2% porosity. The sintered reinforced product was then hot-worked in accordance with the invention for the reasons given in Example V.

The strongest structure in the reinforced product of the invention is one in which the slip and recovery inhibitor phase is extremely small, for example, whose average size is less than two microns and preferably even less than one micron, and in which the phase is uniformly distributed throughout the metal matrix in a substantially discontinuous random fashion. For optimum mechanical properties, it is desired that the average spacing between the slip inhibitor phase should be less than one micron and preferably fall within the range of about 0.1 to 0.5 micron. If the average distance is greater than one micron the properties fall off appreciably and if the average distance is less than 0.1 micron the product may be brittle or the hard phase may dissolve in subsequent heating treatments and lose its stability.

As illustrative of the structures which are obtained with the reinforced product, reference is made to Figs. 1 and 2 of the drawing. Fig. 1 depicts the structure at 4000 times magnification of the reinforced product of the invention comprising about 7% by weight of titanium carbide distributed as an extremely small phase in a substantially discontinuous, random fashion through a matrix alloy of about 80% nickel and 20% chromium comprising about 93% by weight of the reinforced

product. Fig. 2 is the same magnification as Fig. 1 except it depicts a structure containing about 10% by weight of the substantially insoluble titanium carbide slip inhibitor phase distributed through the same matrix alloy.

In evaluating the capability of the reinforced product of the invention to sustain itself under stress at elevated temperatures, a short time high temperature tensile test is employed. The test comprises heating a tensile test specimen to an elevated temperature, say 1000° C., and determining its ultimate strength at that temperature in the conventional manner. In this way the reinforced product of the invention can be compared to a similar product produced by conventional methods. Tests have shown an 80-20 nickel-chromium alloy containing no TiC softens appreciably above 850° C. and generally has unsatisfactory resistance to creep at 950° C. and high temperatures. Even if the alloy contains elemental titanium and/or aluminum as age hardeners, the alloy softens due to overaging at 850° C. and higher and solution softens at 950° C. and higher when held at these temperatures for prolonged periods of time. In either case the alloy suffers in its creep properties and may be unsatisfactory. However, when the alloy is reinforced by at least about 5% and up to about 20% by volume of the inhibitor material in accordance with the invention, e. g. with titanium carbide, the alloy exhibits improved resistance to creep and is able to sustain itself under stress at a temperature range between 850° C. and 1050° C. for prolonged periods of time. When the alloy contains substantially less than 5% by volume of the slip and recovery inhibitor, the properties are not sufficiently improved in accordance with the invention. Likewise, when the alloy contains substantially more than 20% by volume of the inhibitor phase, the alloy loses its ductility and exhibits low resistance to impact.

As has been stated before, the novel results can only be achieved by employing powder metallurgy as the processing method for producing the reinforced metal product of the invention. This enables the use of large amounts of slip inhibitor compound material in amounts up to about 20% by volume of the product (or up to about 15% by weight). Thus, a nickel-chromium reinforced product containing about 15% by weight of titanium carbide would in effect contain about 12% by weight of titanium and about 3% by weight of carbon. If the same nickel-chromium product was produced by regular melting and casting procedures it would be necessary to add an equivalent of 12% titanium and 3% carbon. The alloy would be brittle and substantially unworkable. Furthermore, the titanium carbide in the cast product would be in the form of a substantially continuous dendritic phase and would not be homogeneous and evenly dispersed as fine particles as in the case of the reinforced metal product of the invention. Such a cast material would also have a very low resistance to impact. The product of the invention maintains a rather high resistance to impact even when it contains large amounts of the slip inhibitor material provided the slip inhibitor phase is uniformly dispersed throughout the matrix.

While it has been shown that substantially stable reinforced metal products of high strength can be produced from relatively soft nickel-chromium alloys of the 80-20 nickel-chromium type alloy, it will be appreciated that other types of heat resistant alloys can be reinforced, including the age-hardenable nickel and cobalt-base alloys. Thus, the slip inhibitor can be used in conjunction with these alloys to further augment their weight carrying capacity at elevated temperature. In other words, as the age hardening alloys lose their load carrying capacity at the high temperatures, the slip and recovery inhibitor phase takes over and helps to sustain the strength of the alloy.

Although the present invention has been described in conjunction with preferred embodiments, it is to be

understood that modifications and variations may be resorted to without departing from the spirit and scope of the invention, as those skilled in the art will readily understand. Such modifications and variations are considered to be within the purview and scope of the invention and appended claims.

We claim:

1. A method for reinforcing heat resistant metal products capable of sustaining high strength properties and high resistance to creep at elevated temperatures above 800° C. and up to about 1050° C. for prolonged periods of time which comprises uniformly mixing about 5% to 20% by volume of a finely divided powder of a slip and recovery inhibiting compound phase having a particle size not exceeding about 10 microns selected from the group consisting of carbides, borides, silicides and nitrides of titanium, zirconium, columbium, tantalum, vanadium and hafnium, and disilicides of molybdenum and tungsten, with a finely divided heat resistant matrix metal powder not exceeding about 40 microns in size to make up substantially the balance, said heat resistant matrix metal comprising by weight about 5% to 30% chromium, up to about 25% iron with substantially the remainder of the matrix metal being at least one metal selected from the group consisting of up to about 90% nickel and up to about 70% cobalt, the sum of the nickel and cobalt contents being at least about 40% by weight of the matrix metal composition, shaping said powder mixture to a coherent body, sintering the shaped body at a temperature of at least about 1100° C. to not greater than about 5° C. below the point of incipient fusion at a subatmospheric pressure not exceeding about 100 microns to produce a substantially dense body, hot working said sintered body to reduce its cross-sectional area at least about 50% to eliminate substantially the voids in said body and to effect optimum dispersion of said slip and recovery inhibiting phase, and then fabricating said hot worked body into a heat resistant article of manufacture, said fabricated article being characterized by a micro-structure having a substantially discontinuous and random dispersion of the finely divided slip and recovery inhibiting phase throughout the matrix of the heat resistant metal, the average distance between the finely divided phase being not greater than about one micron.

2. A method for reinforcing heat resistant metal products capable of sustaining high strength properties and high resistance to creep at elevated temperatures above 800° C. and up to about 1050° C. for prolonged periods of time which comprises uniformly mixing about 5% to 20% by volume of a finely divided powder of a slip and recovery inhibiting compound phase having a particle size not exceeding about 2 microns selected from the group consisting of carbides, borides, silicides and nitrides of titanium, zirconium, columbium, tantalum, vanadium, and hafnium, and disilicides of molybdenum and tungsten, with a finely divided heat resistant matrix metal powder not exceeding about 5 microns in size to make up substantially the balance, said heat resistant matrix metal comprising by weight about 5% to 30% chromium, up to about 25% iron with substantially the remainder of the matrix metal being at least one metal selected from the group consisting of up to about 90% nickel and up to about 70% cobalt, the sum of the nickel and cobalt contents being at least about 40% by weight of the matrix metal composition, shaping said powder mixture to a coherent body, sintering the shaped body first at a temperature of about 1100° C. to 1125° C. at a subatmospheric pressure not exceeding about 50 microns of mercury column followed by a second sintering at a temperature of 5° C. to 100° C. below the point of incipient fusion at a subatmospheric pressure not exceeding about 0.1 micron of mercury column to produce a substantially dense body, hot working said sintered body to reduce its cross-sectional area to at least about 50% to eliminate substantially the voids in said body and to effect optimum

dispersion of said slip and recovery inhibiting phase, and then fabricating said hot worked body into a heat resistant article of manufacture, said fabricated article being characterized by microstructure having a substantially uniform dispersion of the finely divided slip and recovery inhibiting phase throughout the matrix of the heat resistant metal, the average distance between the finely divided phase being not greater than about one micron.

3. A method for reinforcing heat resistant metal products capable of sustaining high strength properties and high resistance to creep at elevated temperatures above about 800° C. and up to about 1050° C. for prolonged periods of time which comprises uniformly mixing about 5% to 20% by volume of a finely divided powder of a slip and recovery inhibiting compound phase having a particle size not exceeding about 1 micron selected from the group consisting of carbides, borides, silicides and nitrides of titanium, zirconium, columbium, tantalum, vanadium, and hafnium, and disilicides of molybdenum and tungsten, with a finely divided heat resistant matrix metal powder not exceeding about 5 microns in size to make up substantially the balance, said heat resistant matrix metal comprising by weight of about 5% to 30% chromium, up to about 25% iron with substantially the remainder of the matrix metal being at least one metal selected from the group consisting of up to about 90% nickel and up to about 70% cobalt, the sum of the nickel and cobalt contents being at least about 50% by weight of the matrix metal composition, shaping said powder mixture to a coherent body in a mold under a pressure of at least about 30 t. s. i., sintering the shaped body first at a temperature of about 1100° C. to 1125° C. at a subatmospheric pressure not exceeding 50 microns of mercury column followed by a second sintering at a temperature of about 25° C. to 100° C. below the point of incipient fusion at a subatmospheric pressure not exceeding about 0.1 micron of mercury column to produce a substantially dense body, hot working said sintered body to reduce its cross-sectional area to at least about 90% to eliminate substantially the voids in said body and to effect optimum dispersion of said slip and recovery inhibiting phase, and then fabricating said hot worked body into a heat resistant article of manufacture, said fabricated article being characterized by micro-structure having a substantially discontinuous and random dispersion of the finely divided slip and recovery inhibiting phase throughout the matrix of the heat resistant metal, the average distance between the finely divided phase being of the order of about 0.1 to 0.5, micron.

4. A method for reinforcing heat resistant metal products capable of sustaining high strength properties and high resistance to creep at elevated temperatures above 800° C. and up to about 1050° C. which comprises uniformly mixing about 5% to 20% by volume of a finely divided powder of a slip and recovery inhibiting compound phase comprising titanium carbide having a particle size not exceeding about 1 micron with a finely divided heat resistant matrix metal powder not exceeding about 5 microns in size to make up substantially the balance, said heat resistant matrix metal comprising by weight about 5% to 30% chromium, up to about 25% iron with substantially the remainder of the matrix metal being at least one metal selected from the group consisting of up to about 90% nickel and up to about 70% cobalt, the sum of the nickel and cobalt contents being at least about 50% by weight of the matrix metal composition, shaping said powder mixture to a coherent body in a mold under a pressure of about 30 to 150 t. s. i., sintering the shaped body first at a temperature of about 1100° C. to 1125° C. at a subatmospheric pressure not exceeding about 50 microns of mercury column followed by a second sintering at a temperature of about 25° C. to 100° C. below the incipient point of fusion at a subatmospheric pressure not exceeding about 0.1 micron to produce a substantially dense body, hot working said sintered body to

reduce its cross-sectional area to at least about 90% to eliminate substantially the voids in said body and to effect optimum dispersion of said slip and recovery inhibiting phase, and then fabricating said hot worked body into a heat resistant article of manufacture, said fabricated article being characterized by microstructure having a substantially discontinuous and random dispersion of the finely divided slip and recovery inhibiting phase comprising titanium carbide throughout the matrix of the heat resistant metal, the average distance between the finely divided phase being of the order of about 0.1 to 0.5 micron.

5. A method for reinforcing heat resistant metal products capable of sustaining high strength properties and high resistance to creep at elevated temperatures above 800° C. and up to 1050° C. for prolonged periods of time which comprises uniformly mixing about 5% to 20% by volume of a finely divided powder of a slip and recovery inhibiting compound phase selected from the group consisting of carbides, borides, silicides, and nitrides of titanium, zirconium, columbium, tantalum, vanadium and hafnium, and disilicides of molybdenum and tungsten, with a finely divided heat-resistant matrix metal powder to make up substantially the balance, said heat resistant matrix metal comprising by weight about 5% to 30% chromium, up to about 25% iron with substantially the remainder of the matrix metal being at

10 least one metal selected from the group consisting of up to about 90% nickel and up to about 70% cobalt, the sum of the nickel and cobalt contents being at least about 40% by weight of the matrix metal composition, shaping said powder mixture to a coherent body, sintering the shaped body at a temperature of at least about 1100° C. at a subatmospheric pressure not exceeding about 100 microns to produce a substantially dense body, hot working said sintered body to reduce its cross-sectional area at least about 50% to eliminate substantially the voids in said body and to effect optimum dispersion of said slip and recovery inhibiting phase, and then fabricating said hot worked body into a heat resistant article of manufacture, said fabricated article being characterized by a microstructure having a substantially discontinuous and random dispersion of the finely divided slip and recovery inhibiting phase throughout the matrix of the heat resistant metal, the average distance between the finely divided phase being not greater than about one micron.

20

## References Cited in the file of this patent

## UNITED STATES PATENTS

|           |                 |                |
|-----------|-----------------|----------------|
| 2,106,162 | Balke           | Jan. 25, 1938  |
| 2,174,025 | Wise et al.     | Sept. 26, 1939 |
| 2,580,171 | Hagglund et al. | Dec. 25, 1951  |
| 2,686,118 | Cavanagh        | Aug. 10, 1954  |